

## UNITED STATES PATENT OFFICE.

SAMUEL PEACOCK, OF WHEELING, WEST VIRGINIA, ASSIGNOR TO WHEELING STEEL CORPORATION, OF WHEELING, WEST VIRGINIA, A CORPORATION OF DELAWARE.

### RUST-RESISTING MILD STEEL AND PROCESS OF PRODUCING THE SAME.

No Drawing.

Application filed March 14, 1924. Serial No. 699,315.

To all whom it may concern:

Be it known that I, SAMUEL PEACOCK, a citizen of the United States, residing at Wheeling, in the county of Ohio and State of West Virginia, have invented certain new and useful Improvements in Rust-Resisting Mild Steel and Processes of Producing the Same; and I do hereby declare the following to be a full, clear, and exact description 10 of the invention, such as will enable others skilled in the art to which it appertains to make and use the same.

This invention relates to a rust resisting iron or steel and process of producing the same, and has for its object to improve the procedures and the products of this nature which have been heretofore proposed.

With these and other objects in view, the invention consists in the novel steps and combinations of steps constituting the process and in the novel iron or steel product constituting the product, all as will be more fully hereinafter disclosed and particularly pointed out in the claim.

It is well known that the presence of a small percentage of copper in mild steel, say, from 0.1% to 0.3%, will increase its resistance to corrosion when exposed to acid solutions or solutions carrying ionizable salts. But it is also well known that in alkaline solutions or in water of a high degree of purity, the presence of such small percentage of copper will increase the velocity 30 of the corrosion of said steel.

In this invention, on the other hand, I

have found that when a like small percentage of tin is added to the said copper bearing mild steel, the resulting metal not only retains its resistance to the corrosion of acid solutions and solutions of ionizable salts, 40 but it also possesses an equal measure of resistance to the corrosion to alkaline solutions and to water of a high degree of purity. That is, if a mild steel in its molten state is treated with not more than 0.3% and not 45 less than 0.1% of copper, and like quantities of tin, or if said quantities of copper and tin are otherwise alloyed therewith, the resulting product will possess an increased 50 resistance to corrosion from solutions of acids, solutions of ionizable salts, alkaline solutions and water of a high degree of purity. On the other hand, if the quantities of copper and tin be increased or diminished beyond the limits stated inferior results will 55 be encountered.

I am unable to give a satisfactory scientific explanation of the coaction of the tin and copper, and believe it is due to some unexplained inter-ionic action between the tin 60 and copper in the presence of the iron which inhibits the oxidation of the iron.

What is claimed is:—

The herein described mild steel of a high 65 corrosion resistance, the same containing not less than 0.1% and not more than 0.3% of each of the metals copper and tin.

In testimony whereof I affix my signature.

SAMUEL PEACOCK